

## UNITED STATES PATENT OFFICE.

WILLIAM J. DIEDERICHS AND ANSON HAYES, OF AMES, IOWA.

## PROCESS FOR TREATING IRON.

No Drawing. Original application filed August 21, 1922, Serial No. 583,370. Divided and this application filed August 6, 1925. Serial No. 48,625.

To all whom it may concern:

Be it known that we, WILLIAM J. DIEDERICHS and ANSON HAYES, citizens of the United States of America, and residents of Ames, Story County, Iowa, have invented a new and useful Process for Treating Iron, of which the following is a specification.

The subject matter of this application was originally included in but has been divided 10 from our application filed August 21, 1922, Serial Number 583,370.

The object of this invention is to provide a new and improved process for treating white cast iron whereby an iron is produced 15 having as great or greater tensile strength than white cast iron and also capable of being bent and stretched to a considerable degree before breaking.

This and other objects of the invention 20 will be more clearly pointed out in the specification and set forth in the appended claims.

Any suitable type or form of furnace or so-called annealing oven may be employed 25 in carrying out our improved process, and may be heated by any of the well known fuels such as gas, oil or powdered coal burned in connection with air; or the heat may be secured electrically or by a combination 30 of combustion and electricity, or in any other manner that may be desired so long as the desired temperatures and atmospheres are secured.

The iron used in this process is known 35 as white cast iron, differing principally from ordinary gray iron in that while both contain carbon, the white cast iron contains the carbon principally or wholly in the form of carbide of iron represented by the formula 40  $Fe_3C$ , while gray cast iron contains the carbon to a greater degree in the form of graphite or graphitic carbon.

Through the use of this process we obtain 45 a product having as high or higher tensile strength than white cast iron and under certain conditions of procedure also having considerable ductility or ability to bend and stretch, and which is very useful for certain purposes.

50 In carrying out our improved process we do not of necessity pack the white iron castings in boxes or pots containing the packing material, as is done in the ordinary

malleableizing process as referred to in our parent application above identified. However this may be done at times if desired, but by omitting it considerable time may be saved. When the packing is omitted the white iron castings may be supported in any suitable manner in the furnace to prevent 60 sagging and warping under the intense heat.

The process consists in heating for any length of time, raising the temperature of the white iron castings with convenient 65 rapidity, either rapidly or slowly, to any point between the critical temperature of the material (about 740 degrees centigrade) and the point of incipient fusion, and holding at the chosen high temperature for a period 70 of fifteen minutes to five hours, or more. The actual time required will depend upon the temperature chosen, lower temperatures requiring longer times, and upon the chemical composition of the white iron being 75 treated.

In any case it is only desired to maintain the high temperature until the massive cementite is practically all absorbed in the solid solution. We are satisfied that in most instances it would avail 80 little to hold at the high temperature for a longer period than about five hours, since practically all of the desirable change would have occurred in that time, especially if the high temperature employed is above 900 85 degrees centigrade; and that holding for longer periods would result only in waste of time without corresponding benefit. If a high temperature of less than about 900 degrees centigrade is used the time required to 90 practically complete the absorption of massive cementite into the solid solution will be very materially increased.

The castings are then removed from the furnace and cooled by quenching in any 95 suitable material such as sand, cement, powdered mica or the like, or in any manner outside or inside the furnace, whereby the temperature is reduced to a point considerably below the critical. These operations may then be repeated for any desired number of repetitions, that is to say, the material may be alternately heated to a point above the critical temperature and then cooled to a temperature considerably below 100 the critical. The number of repetitions or

alternate heatings and coolings, as well as the rates of heating and cooling, may be varied in accordance with the properties desired in the product.

6. It has been demonstrated that the resultant product is an iron possessing a strength equal to or considerably greater than the white iron castings and also having a considerable degree of ductility. The variations in the treatment of the material result in castings possessing (1) a high tensile strength, of 85,000 to 90,000 pounds per square inch with no ductility; to (2) those having a strength of say 50,000 to 85,000 pounds per square inch, or more, with two to eight per cent elongation, or more.

When speaking of the critical temperature of the material, the fact should be borne in mind, which is well known in metallurgy, that the critical temperature can be, and is, undercooled by a rapid cooling of the material, and therefore will be reduced by heating to a temperature above the critical and cooling rapidly; so that in 25 thereafter heating to the critical temperature, it is obvious that a lower actual temperature will be involved. The language of this specification and the appended claims is used with this fact in mind and should 30 be so construed.

The particular characteristic of the present invention and process, which distinguishes it from another covered by a copending application, is that in the present 35 instance the cooling, after each heating to a point above the critical temperature, is continued until comparatively low temperatures are reached, and such cooling may be accomplished by any suitable method, either inside or out side the furnace, by cooling in any suitable manner such as by quenching or otherwise.

As an example of our experiments and to illustrate what we have done, we recite the 45 following: Castings of white iron were heated to 900 degrees centigrade for seven hours and were then quenched in oil, after which they were reheated to 700 degrees centigrade for twenty hours, and cooled to 50 room temperature. This last cooling may be at any desired rate faster than about seven degrees per hour. The product showed a tensile strength of 54,000 pounds per square inch with ten per cent elongation, in 55 two inches.

Likewise by way of illustration, samples of white cast iron were heated to 900 degrees centigrade for five hours, cooled in sand to room temperature, reheated to 810 degrees 60 centigrade and held for one hour, then cooled at the rate of two degrees per minute to 650 degrees centigrade. The tensile strength was 72,000 pounds per square inch and elongation six per cent.

65 Likewise bars of white cast iron were

alternately heated to a temperature between about 800 and 850 degrees centigrade and cooled in sand, but the final cooling being with the furnace. The heating to 850 degrees was carried out for various numbers of 70 repetitions, with varying results. After seventeen such heatings the product showed a tensile strength of 84,700 pounds per square inch with five and one-half per cent elongation in two inches; and after nineteen such heatings the tensile strength was 82,900 pounds per square inch with six per cent elongation. 75

We claim as our invention:—

1. The process for the heat treatment of 80 castings from white cast iron which consists in (1) subjecting the casting to a temperature above the critical temperature of the material; (2) cooling the casting to a point considerably below the original critical 85 temperature; (3) reheating the casting to a sufficient temperature to allow structural and chemical changes to progress; and (4) cooling the casting.

2. The process for the heat treatment of 90 castings from white cast iron which consists in (1) subjecting the casting to a temperature above the critical temperature of the material; (2) cooling the casting to a point considerably below the original critical 95 temperature; (3) reheating the casting to a sufficient temperature to allow structural and chemical changes to progress; (4) cooling the casting; and (5) a repetition of steps 100 (3) and (4) alternately.

3. The process for the heat treatment of 105 castings from white cast iron which consists in (1) the subjecting of the casting to a temperature above the critical temperature of the material; (2) the cooling of the casting to a point considerably below the original critical temperature by quenching; (3) reheating the casting to a sufficient temperature to allow structural and chemical 110 changes to progress; (4) cooling to a temperature sufficiently low that structural and chemical changes cease; and (5) a repetition of steps (3) and (4).

4. The process for the heat treatment of 115 castings from white cast iron which consists in (1) the subjecting of the casting to a temperature above the critical temperature of the material; (2) the cooling of the casting to a point considerably below the original critical temperature by quenching; (3) reheating the casting to a sufficient temperature to allow chemical and structural 120 changes to progress; and (4) cooling the casting to a temperature sufficiently low that chemical and structural changes cease. 125

5. The process for the heat treatment of 130 castings from white cast iron which consists in (1) the subjecting of the casting to a temperature considerably above the critical temperature of the material for a period of

from fifteen minutes to five hours, or more, changes cease, at a rate not less than about seven degrees centigrade per hour. <sup>10</sup>  
until the iron carbide present is practically all absorbed in the solid solution, or in other words until in irons of commercial composition the combined carbon is reduced to substantially nine-tenths of one per cent; and (2) the cooling of the casting to a temperature where chemical and structural

Signed at Des Moines, in the county of Polk and State of Iowa, this 18th day of June, 1925.

WILLIAM J. DIEDERICHS.  
ANSON HAYES.